

Patented May 4, 1926.

## UNITED STATES PATENT OFFICE.

WILLIAM PORTER DREAPER, OF LONDON, ENGLAND.

## MANUFACTURE OF ARTIFICIAL SILK AND LIKE MATERIALS FROM VISCOSE SOLUTIONS.

Application filed October 18, 1923. Serial No. 669,281.

No Drawing.

*To all whom it may concern:*

Be it known that I, WILLIAM PORTER DREAPER, a British subject, residing at 27 Willow Road, Hampstead, London, N. W. 3, England, have invented new and useful Improvements in the Manufacture of Artificial Silk and like Materials from Viscose Solutions, of which the following is a specification.

10 In the manufacture of artificial silk, staple fibre and like products by the viscose process, it is usual to use a precipitating bath which consists of a salt such as sodium sulphate to which a certain amount of sulphuric acid has been added, and to add certain other substances such as glucose or zinc chloride or both to improve the spinning qualities and facilitate working conditions, but generally speaking the filaments so produced have not been spun below a size of, say, six to eight deniers from such a bath owing to difficulties being met with in practice, and as a result the general run of filaments produced commercially by the viscose process have approximated to those instanced. Such acid baths as have been mentioned have been used of varying strengths of acid and added salt, and in some cases it has been suggested that very concentrated solutions should be utilized. Such practice introduces difficulties which have generally acted against the use of such solutions.

I now find that the finer filaments can be easily produced even down to from two to four deniers in size without material increase in cost or difficulty in manufacture by introducing into the "acid-salt" precipitating bath a relatively small amount of ammonium sulphate or other salt of ammonia, when it has been observed that the actual formation of the filaments in the bath is so regulated that finer filaments can be drawn off than in the ordinary bath, and yet finally a filament in strand is produced which will readily stand the strain of subsequent operations of winding and treatment to which they are ordinarily subjected. In fact spinning operations are so improved that such fine filaments may even be more easily produced in this bath than the coarser ones in an ordinary "acid-salt" bath.

To illustrate this invention the following example is given. The precipitating bath is made up with say, twenty per cent of sodium sulphate and from seven to fourteen per cent

of sulphuric acid and to this bath is added from one per cent to eight per cent of ammonium sulphate. A bath containing from three to six per cent of ammonium sulphate is particularly useful and when such a bath is kept at a temperature which may vary between 30° C. and 70° C., but preferably about 42° C., fine filaments can be easily spun at a rate of fifty metres per minute or more from holes even up to 0.15 mm. diameter. Such results indicate that in the presence of such relatively small amounts of ammonium salt in the strength of the bath indicated considerably more extension of the forming filaments is possible when this salt is added to an acid bath of the composition named. This bath may also be used in suitable strength in the guider funnel when such is used or the said bath may be immediately followed by a treatment with any other selected solution or even water and then simultaneously passed to and spun into a centrifugal box or collected on a bobbin in the well known manner, or otherwise treated or collected as hitherto.

With this addition to the bath it is not necessary to add glucose or other similar organic substances to the bath or any other addition other than the normal constituents of the bath as mentioned. In addition, and where a separate treatment in the guider funnel is adopted a certain amount of the ammonium salt can be recovered by known means from the guider funnel solution or the wash waters.

I claim:

1. The manufacture of artificial silk and like products of fine filaments from viscose solutions in an "acid-salt" bath of relatively low concentration characterized by containing twenty-two per cent of sodium sulphate, seven to fourteen per cent sulphuric acid, to which is added about five per cent (not being less than one per cent or more than eight per cent) of ammonium sulphate, the said filaments being drawn off at a speed of fifty metres per minute or more.

2. The manufacture of artificial silk and like products of fine filaments from viscose solutions in an "acid-salt" bath of relatively low concentration characterized by containing twenty-two per cent sodium sulphate, twelve per cent sulphuric acid, to which is added six per cent ammonium sulphate.

3. The manufacture of artificial silk and

like products of fine filaments from viscose solutions in an "acid-salt" bath of relatively low concentration characterized by said bath containing twenty-two per cent sodium sulphate or an equivalent acting sulphate, or an equivalent portion of the same which will enable such fine filaments to be produced,

seven to fourteen per cent sulphuric acid, to which is added about five per cent (not being less than one per cent or more than eight per cent) of ammonium sulphate, said filaments being drawn off at a speed of fifty metres per minute or more.

WILLIAM PORTER DREAPER.